

## UNITED STATES PATENT OFFICE

2,166,341

## MACHINABLE PLASTIC ZINC ALLOY

Arthur Burkhardt, Berlin-Lichterfelde, and Wolfgang Wolf, Magdeburg, Germany, assignors to Georg von Giesche's Erben, Breslau, Germany, a corporation of Germany

No Drawing. Application October 25, 1937, Serial No. 170,855. In Germany January 5, 1937

4 Claims. (Cl. 75—178)

Our invention relates to non-ferrous alloys which are suitable for machining on automatic machine tools.

Bar or rod material, in order to be suitable for automatic machine tools, must possess such properties that the tool has long life and a good surface finish is given to the work, but, above all, that the chips are short and spouting.

The only known non-ferrous alloy which possesses these properties is "Ms 58", a brass containing 58 per cent copper, so-called automatic-machine brass.

It is an object of our invention to provide a substitute for Ms 58 which has similar properties.

To this end, we provide an alloy containing 2 to 5 per cent copper, 0.1 to 1 per cent bismuth, 0.1 to 1 per cent manganese, and fine zinc poor in iron and cadmium and practically free from magnesium and tin.

In the search for substitutes for Ms 58, it has been attempted to machine on automatic machines zinc and aluminium alloys of the usual kind. This was a failure because the chips of such alloys are curly and bulky and coil themselves about the tool and the work.

An alloy which is to be a proper substitute for Ms 58 must deliver short and spouting chips on the same machines and under the same cutting conditions as Ms 58, and its finish must not be less perfect nor the life of the tool shorter.

Investigations showed that for obtaining short and spouting chips from a zinc alloy, it is necessary to make additions which in liquid condition are only partly miscible with zinc.

Such additions are lead, thallium, and bismuth. While they had a favorable influence on the formation of the chips, it was found that they were very detrimental with respect to intercrystalline corrosion. Thus, an addition of 0.1 per cent lead or bismuth to the well known die-casting alloy having 4 per cent aluminium, 3 per cent copper, 0.04 per cent magnesium, and zinc as the remainder, caused a growth of more than 7 per cent in length.

The surprising discovery was made that zinc alloys free from aluminium and magnesium, with up to 5 per cent copper, and with addition of lead or bismuth do not suffer from intercrystalline corrosion and possess mechanical properties that they can be used instead of Ms 58.

It was found, however, that the percentage of lead must be 3 to 5 per cent in order to effect the desired formation of short, spouting chips, and this has the drawback of greatly reducing the

ductility of the alloy so that it cannot be worked into bars or rods by extrusion.

Bismuth in amounts of 0.1 to 1 per cent is sufficient for obtaining quite short chips and has a less detrimental influence on ductility, but still the plasticity and the mechanical properties of an alloy of copper and zinc with such percentages of bismuth are such that the alloy can be used in practice but still is not quite satisfactory.

We have made the surprising discovery that by adding 0.1 to 1 per cent manganese to a bismuth-containing copper-zinc alloy its plasticity and mechanical properties are improved, and the properties of its chips are not deteriorated.

The following table gives some examples of alloys embodying our invention.

In all alloys, the remainder or base is fine zinc poor in iron and cadmium and practically free from magnesium and tin.

Composition in per cent

|   | Copper | Bismuth | Manganese |    |
|---|--------|---------|-----------|----|
| 1 | 2      | 0.5     | 0.5       | 25 |
| 2 | 2      | 0.7     | 0.7       |    |
| 3 | 2      | 1       | 0.3       |    |
| 4 | 2      | 1       | 1         |    |
| 5 | 3      | 0.5     | 0.5       |    |
| 6 | 4      | 0.5     | 0.5       |    |
| 7 | 4      | 1       | 0.3       | 30 |
| 8 | 4      | 1       | 1         |    |
| 9 | 5      | 0.7     | 0.7       |    |

Alloy (1) has given the best results with respect to working and to machining in an automatic machine tool. Alloy (6) is very good for purposes where hardness and high tensile strength are required, as it is superior to (1) in these respects but is less ductile.

Iron and cadmium are detrimental to the formation of the chips, and therefore the alloy must be poor in these constituents. The influence of magnesium and tin is still more unfavorable in this respect, and this is why the alloy should be practically free from magnesium and tin.

Alloys altogether without aluminium must not be melted in iron containers, since the zinc strongly attacks the iron. This is prevented by a slight addition of aluminium, up to 0.15 per cent. This amount is not detrimental in other respects and the alloy can now be melted in an iron container.

We claim:

1. A machinable plastic zinc alloy containing from a small but effective amount up to 5 per cent of copper, from 0.1 to 1 per cent of bismuth, 55

- from 0.1 to 1 per cent of manganese, and fine zinc poor in iron and cadmium, and practically free from magnesium and tin, as the remainder.
2. A machinable plastic zinc alloy containing from 2 to 5 per cent of copper, from 0.1 to 1 per cent of bismuth, from 0.1 to 1 per cent of manganese, and fine zinc poor in iron and cadmium, and practically free from magnesium and tin, as the remainder.
- 5 3. A machinable plastic zinc alloy containing from a small but effective amount up to 5 per cent of copper, 0.1 to 1 per cent of bismuth, 0.1 to 1 per cent of manganese, the remainder substantially all zinc, and characterized by resistivity to intercrystalline corrosion in combination with high ductility and the property of producing short and spurting chips when being machined.
- 10 4. A machinable plastic zinc alloy containing 2 to 5 per cent of copper, 0.1 to 1 per cent of bismuth, 0.1 to 1 per cent of manganese, the remainder substantially all zinc, and characterized by resistivity to intercrystalline corrosion in combination with high ductility and the property of producing short and spurting chips when being machined.

ARTHUR BURKHARDT.  
WOLFGANG WOLF.